

Sept. 15, 1936.

M. PIER ET AL.

2,054,776

## CONVERSION OF CARBONACEOUS MATERIALS

Filed Aug. 15, 1933



Bruno Engel  
Walter König and  
Mathias Pier Inventors

By Ch. Young - Attorney

## UNITED STATES PATENT OFFICE

2,054,776

## CONVERSION OF CARBONACEOUS MATERIALS

Mathias Pier, Heidelberg, Bruno Engel, Mannheim, and Walter Kroenig, Ludwigshafen-on-the-Rhine, Germany, assignors to Standard I. G. Company, Linden, N. J., a corporation of Delaware

Application August 15, 1933, Serial No. 685,229  
In Germany August 26, 1932

2 Claims. (Cl. 196—53)

The present invention relates to improvements in the treatment with hydrogenating gases of carbonaceous materials containing or giving rise to the formation of asphalt to produce valuable hydrocarbon products and in particular to an advantageous manner of adding catalysts to the reagents.

The drawing represents in diagrammatic form an apparatus suitable for carrying out the invention.

In the conversion by heat of carbonaceous materials comprising asphalt, i. e. containing or giving rise to the formation of asphalt, such as coals made into pastes with oils or oils containing asphalt, in particular in the presence of hydrogenating gases, and more especially in the destructive hydrogenation of said materials, catalysts have hitherto been added thereto before their entry into the apparatus, the mixture then being brought to the reaction temperature in a preheater. In this process it was observed that during the heating the high molecular asphalt-like constituents of the initial materials penetrate into the pores of the catalyst and thus impair its activity already at the beginning of the reaction. Furthermore the small particles of catalyst become stuck together by the asphalt forming larger particles, which then settle in an undesirable manner. The catalysis thereby suffers owing to the resulting absence in the reaction space of active catalyst due to the setting of large amounts of stuck catalyst which is therefore wasted. The said conglomeration of catalyst may in some cases even take place when a suspension prepared by grinding the catalyst with an oil containing asphalt is allowed to stand for some time while hot.

We have now found that the disadvantages hereinbefore mentioned are avoided by dispersing the catalyst in the absence of asphalt in an oil which is free from asphalt and which when mixed with the carbonaceous material to be treated or the products formed therefrom does not cause flocculation of the asphalt present or formed during the working up and then adding the suspension to the initial material to be treated or undergoing treatment. The term "dispersing" includes suspending or making up into a paste. By the expression "oils not causing flocculation of asphalt" we mean either oils which do not

cause flocculation even when added in large quantities or oils employed in such amounts as do not cause flocculation though larger amounts thereof are capable of causing flocculation. Thus for example also a middle or heavy oil consisting of a large proportion of saturated hydrocarbons may be employed if it is added in but so small quantities that no flocculation takes place. By "asphalts" we understand substances which are chemically similar to natural asphalt and which represent black brown, solid or semi-solid high molecular hydrocarbon compounds containing oxygen and in most cases also sulphur, which are dissolved or suspended in mineral oils or other liquid hydrocarbon products such as products obtained by the destructive hydrogenation of carbonaceous materials and which may in part be precipitated from the said liquid hydrocarbon products by benzine and in part from their solution in ether by addition of alcohol (see Holde 20 "Kohlenwasserstofföle und Fette", 1933, page 164).

The present invention is of particular advantage in processes in which the catalyst dispersion in oil is admixed with the initial materials prior to any heating or preheating necessary to bring them to the reaction temperature. The said heating is preferably carried out with an addition of a hydrogenating gas such as hydrogen.

By stating that the dispersion of the catalyst in an oil free from asphalt should take place in the absence of asphalt we wish to exclude a treatment in which the catalyst is first contacted with an asphalt-containing oil and then further distributed in another oil which may be free from asphalt, since this procedure would result in the preparation of a catalyst which is soon clogged up with asphalts. The pre-treatment of the catalyst in the absence of asphalt with an oil free from asphalt has the result that the capacity of the catalyst for adsorption is practically completely used up by the oil free from asphalt, so that the catalyst, for example during its heating up together with the initial material, has practically no adsorptive capacity for the asphaltic constituents, although the invention is not limited by this theory. It is preferable to add the suspension of the catalyst in the oil free from asphalt to the oil containing asphalt which is to be worked up, at a time which is not too long before the working up, because when the mixture is allowed to stand

for a very long period of time an exchange between the oil free from asphalt on the surface of the catalyst and the oil containing asphalt commences to take place.

5 For the purposes of the present invention an oil is considered to be free from asphalt, if it is entirely or practically free therefrom that is to say, if it does not contain asphalt in amounts above 0.5 per cent and preferably not above 0.3 10 per cent by weight. The amount of asphalt contained in the oil as defined in the present specification is determined as follows:

15 2 grams of oil are mixed with 5 cubic centimeters of benzene and 100 cubic centimeters of normal benzene, and allowed to stand for 12 hours. The asphalt which precipitates out is filtered off, washed on the filter with normal benzene and dissolved in benzene. The benzene is evaporated off, and the residual asphalt is dried and weighed. 20 20 As oils free from asphalt may be mentioned middle oils or heavy oils answering to said specification and it is particularly advantageous to employ a heavy oil answering to said specifications obtained by destructive hydrogenation from the initial materials to be worked up. Thus middle oils or heavy oils obtained by the destructive hydrogenation of mineral coals or mineral coal tars are of advantage as oils free from asphalts to be pasted up with the finely divided catalysts. Also fractions of these tars themselves are suitable for this purpose. As further examples of such oils may be mentioned anthracene oil free from asphalt or oils, preferably of middle oil boiling point range, obtained by the destructive hydrogenation of carbonaceous materials at temperatures of the upper half of the temperature range suitable for this reaction, whereby a high content of aromatic hydrocarbons is imparted to the final products. Also naphthenic or paraffinic base oils come into 30 question, the latter being employed in such small quantities that no flocculation takes place. It is of advantage to select an oil as dispersing medium which has a gravity of the order of the catalyst to be dispersed or previously to intimately mix the catalyst to be dispersed in the oil with a solid substance which adapts the gravity of the solid mixture to that of the oil in which it is to be dispersed.

35 These oils, when not added in restricted amounts, should not contain so much aliphatic constituents rich in hydrogen that there is any danger when mixing these oils with an asphalt containing oil that a flocculation of the asphalt which would lead to clogging of the apparatus, occurs. As a rule not more than 20 per cent, preferably less than 15 per cent, of aliphatic constituents rich in hydrogen reckoned on the initial material comprising asphalt should be added to the latter.

40 The invention is of particular importance for working up tars or mineral oils containing asphalt, fractions of high boiling point of the same or coals of all varieties made into pastes with oils which yield oils containing asphalt during their working up, as for example mineral coal or lignite. Peats, shales or shale oils, tar sands and their distillation products containing or giving rise to the formation of asphalt may be worked up with advantage. Even oils containing more 45 than 30 per cent of asphalt may be advantageously treated in accordance with the present invention.

50 As catalysts may be mentioned those having a hydrogenation action, especially metals, or their compounds, of the 2nd to the 8th group of the

5 periodic system, as for example zinc, magnesium, cadmium, boron, titanium, tin, lead, vanadium, manganese, iron, cobalt, rhenium and especially those of the 6th group, such as chromium, molybdenum, tungsten and uranium. Advantageous compounds are oxides and sulphides. The catalysts may also be precipitated on carriers, such as Florida earth, active silica, kieselguhr, active carbon, coke or brown coal small coke, preferably neutralized with acid, and, if desired, activated with steam. The preparation of such catalysts may be effected for example by impregnating or sprinkling the carrier with the catalyst solution. For example an aqueous solution of a molybdate or tungstate, or tin oxalate dissolved in ammonium oxalate solution, or molybdenum heptachloride, molybdic acid chloride or tungsten hexachloride dissolved in naphthenic acid or oleic acid, may be employed. The catalytic material may also be brought on to the carrier substance while it is in a colloidal state of dispersion.

10 The expression "treatment by heat, preferably with hydrogenating gases" where herein employed is intended to comprise the most various reactions. The said treatment may be used to produce hydrocarbons of all sorts by cracking or by destructive hydrogenation, such as motor fuels, middle oils, kerosene and lubricating oils. The said expression also includes the removal of non-hydrocarbon impurities, such as sulphur- 15 or oxygen-containing substances or nitrogen compounds by the action of hydrogen or gases containing or supplying hydrogen from crude carbonaceous materials containing or giving rise to asphalt, for example the refining by treatment with hydrogen of crude benzol containing asphalt, of crude motor fuels or of lubricating oils, containing or giving rise to asphalt. The said expression further includes the conversion of oxygen or sulphur containing organic compounds containing or giving rise to asphalts to produce the corresponding hydrocarbons or hydrogenated hydrocarbons, for example the conversion of phenols or cresols containing asphaltic substances into the corresponding cyclic hydrocarbons or hydrogenation 20 products thereof. Finally it includes the hydrogenation of unsaturated compounds containing asphalt and more particularly of unsaturated hydrocarbons of said nature or of aromatic compounds containing asphalt and more particularly of aromatic hydrocarbons of said nature, for example, to produce hydroaromatic hydrocarbons.

25 The said reactions by heat treatment, especially with hydrogen or hydrogen containing gases, are effected in the liquid phase and usually carried out at temperatures between 250° and 700° C., usually between 300° and 700° C. and more preferably between 380° and 550° C. The pressures employed may be atmospheric or superatmospheric; they are preferably in excess of 20 atmospheres and more advantageously in excess of 50 atmospheres. In some reactions, however, for example, in the refining of crude benzol containing asphalt, rather low pressures, for example, of the order of 40 atmospheres may be employed. Generally, however, pressures of about 100, 200, 300, 500 and in some cases even 1000 atmospheres come into question.

30 The amount of hydrogen maintained in the reaction space and parts connected therewith, if any, varies greatly with the nature of the particular initial materials treated or according to the result in view. In general 400, 600, 1000 cubic meters or more of hydrogen, measured under normal conditions of temperature and pressure, per 35

ton of carbonaceous material treated may be used. It is particularly advantageous to operate by continuously introducing fresh carbonaceous material into the reaction vessel and to continuously remove products therefrom. If desired several reaction vessels may be employed in which different conditions of temperature and/or pressure may, if necessary, be maintained and in which different catalysts may also be employed. 5 Sufficiently converted reaction products may be removed behind any of the reaction vessels. Materials which have not been sufficiently reacted on may be recycled or treated in a further reaction vessel. The subsequent stages may, if desired, be carried out in the gaseous phase, for example to produce anti-knock motor fuels. One of the subsequent stages may also take the form of a cracking.

Referring to the drawing, numeral 1 indicates 20 a tank in which a catalyst is produced either in solution or in suspended form, as seems desirable. Line 2 conducts this solution or suspension into a mixing chamber 3 into which a carrier material may be placed. The mixing device is fitted 25 with a stirring mechanism and air is injected by means of a line 5 into the catalyst in order to spray the solution or suspension over the carrier material.

The mixing device is also fitted with a chute 30 6 for discharging the catalyst after it has been produced in a dry form into a mixing chamber 7. Asphalt free oil of the types mentioned above, such as anthracene oil, is fed into the mixing chamber from a storage vessel 8a and this mixture is then passed into a disintegrator 8. A pump 9 may be utilized to pass the material discharged from the disintegrator back to the mixing chamber by pipe 10 in order to gain uniformity and a portion thereof may be drawn off by a 35 pipe 11 and discharged into a second mixing chamber 12 which is also fitted with a stirrer 13 and into which a main body of the oil to be subjected to the hydrogenating treatment is conducted by a line 14 from storage 15. The admixture of the three ingredients, namely the catalyst, the asphalt free oil and the oil to be treated, is then passed by a line 16 and pump 17 to a pre-heater 18. Hydrogen is introduced preferably 40 into the inlet of the preheater by means of a pipe 19 and the preheated mixture is passed into a reaction chamber 20. The reaction products may be withdrawn from the top of the reaction chamber by a line 21 and discharged into a separating vessel 22. Liquid and solid materials can be 45 withdrawn by pipe 23 while the vapors pass overhead by a pipe 24 to a condenser 25 and a separating vessel 26 from which gases are removed by 50 27 and the liquefied product by 28.

The expression "hydrogenating gases" means, 55 where herein employed, hydrogen alone or gases containing or supplying hydrogen, for example a mixture of hydrogen with nitrogen, or water gas, or hydrogen mixed with carbon dioxide, hydrogen sulphide, water vapor or methane or other hydrocarbons. Or the hydrogen may be generated in 60 the reaction chamber by the interaction of water and coal, carbon monoxide, hydrocarbons and the like.

The catalysts are preferably admixed with an 65 oil free from asphalt in such amounts that the resulting paste is sufficiently fluid to be easily pumped and homogeneously mixed with the initial material. In general pastes containing between 10 and 60 per cent by weight of catalytic 70 material have proved to be suitable.

Advantageously so much of the catalyst dispersion is admixed with the carbonaceous material that the final mixture contains between 0.05 and 5 per cent by weight and preferably between 0.1 and 1.5 per cent of catalyst relative to the carbonaceous material present. 5

The following examples will further illustrate the nature of this invention but the invention is not restricted to these examples.

10

#### Example 1

Brown coal small coke which has been activated with steam at 900° C. is impregnated with an ammoniacal solution of molybdate acid so that the coke contains 2 per cent of molybdate acid. The catalyst thus prepared is then ground to colloidal fineness in a percussion cross mill and mixed with such an amount of a heavy oil free from asphalt (obtained as hereinafter described) 15 that a suspension containing 30 percent of catalyst is obtained. This mixture of oil and catalyst has added thereto a German petroleum boiling above 325° C. and containing asphalt so that the latter contains 1 per cent of catalyst. The mixture is then heated to 475° C. with hydrogen under a pressure of 200 atmospheres and led through a reaction vessel; 1650 cubic meters of hydrogen are used for each metric ton of oil. The products leaving the reaction vessel are led 20 into a separating vessel kept at 460° C. in which a liquid level is maintained. From the bottom of the vessel are withdrawn 6 per cent (calculated with reference to the treated material) of high boiling products containing catalyst, while the remainder of the reaction products together with the hydrogen are supplied to a fractionating column. From this column are obtained 55 per cent 25 of constituents boiling up to 325° C., which consist of 27 per cent of benzene and 73 per cent of middle oil, and 45 per cent of constituents boiling above 325° C. which are free from asphalt. A part of the latter are employed, as already mentioned, for mixing with the catalyst. The remainder may be supplied to the same or another reaction vessel for further conversion into 30 constituents of lower boiling point. 35

If the catalyst is directly added to the asphaltic initial oil to be converted the catalyst particles become soon stuck together and the catalyst deposits in substantial quantities in the preheater 50 and in the reaction vessel, whereby inconveniences such as a decrease in the activity of the catalyst, a decrease of the volume of the reaction space and a clogging up of the preheating coils are encountered after some time of operation. 55

#### Example 2

Active carbon is impregnated with 5 per cent of zinc chloride and then mixed with a lubricating oil, free from asphalt, obtained from a German mineral oil by distillation or by destructive hydrogenation in such an amount that a suspension containing 30 per cent of catalyst is formed. This suspension is thereupon added to an oil fraction containing asphalt and boiling above 325° C. which is obtained from a German mineral oil, in such an amount that the mixture contains 1 per cent of catalyst. This mixture is then heated in a heating tube system under a pressure of 50 60 atmospheres to 485° C. and subsequently passed through a cracking space connected with said tube system and having a greater diameter than the tubes of this system. In this manner benzene is obtained in a yield of 42.8 per cent with ref- 65 70 75

erence to the initial asphalt containing oil. If the catalyst is directly added to this oil the inconveniences described in Example 1 are encountered.

5 What we claim is:—

- 5 1. In a process of destructive hydrogenation of carbonaceous materials rich in asphalts or substances which produce asphalt during the treatment, the steps of first dispersing a finely divided catalytic material in an oil free from asphalt and which when mixed with the carbonaceous material to be treated or the product formed therefrom does not cause flocculation of asphalt ini-

tially present or formed during the process to form a paste containing 10 to 60% of catalyst, adding the suspension thus formed to the carbonaceous material to be treated, to form a mixture containing from .05 to 5% of catalyst, and then subjecting the mixture to destructive hydrogenation.

6 2. Process according to claim 1 in which the proportion of the catalyst is .1 to 1.5% of the oil mixture.

10 MATHIAS PIER.  
BRUNO ENGEL.  
WALTER KROENIG.